

March 10, 1942.

A. A. NEW  
ELECTRIC INSULATING MATERIAL AND TO CONDUCTORS  
INSULATED WITH SUCH MATERIAL  
Filed Feb. 11, 1938

2,276,084



BY

INVENTOR  
ARCHIBALD ALAN NEW

*Paul R. Adams*  
ATTORNEY

Patented Mar. 10, 1942

2,276,084

# UNITED STATES PATENT OFFICE

2,276,084

## ELECTRIC INSULATING MATERIAL AND TO CONDUCTORS INSULATED WITH SUCH MATERIAL

Archibald Alan New, London, England, assignor to International Standard Electric Corporation, New York, N. Y.

Application February 11, 1938, Serial No. 190,031  
In Great Britain February 26, 1937

2 Claims. (Cl. 174—29)

Esters of cellulose have frequently been proposed for use as electric insulating materials, both in the form of threads spun from such esters and in the form of native cellulose such as cotton or paper that has been partially esterified.

In British Patents 372,312 and 395,737 there are described the partial esterification of cotton and paper up to the mono-acetate stage or in some cases up to the di-acetate stage. Such partially esterified materials possess a comparatively slight increase in electric resistance under dry conditions but a very considerable increase in electric resistance under humid conditions when measured with direct current and compared with the resistance of the corresponding unesterified cellulosic materials.

Cellulose that has been esterified up to the mono-acyl stage was found to show a great improvement under humid conditions in power factor when measured with alternating current of power frequencies. This improvement, however, rapidly decreased with increase of frequency as will be clear from the following table showing the power factor of different forms of cellulose at different frequencies. All the figures relate to cellulose yarns at 60% relative humidity and a temperature of 25° C.

|                                                            | 50 cycles | 400 cycles | 800 cycles | 1000 cycles |
|------------------------------------------------------------|-----------|------------|------------|-------------|
| Washed cotton.....                                         | 0.290     | 0.100      | 0.080      | 0.070       |
| Acetylated cotton of 29% combined acetic acid content..... | 0.024     | 0.015      | 0.009      | 0.005       |
| Acetylated cotton of 55% combined acetic acid content..... | 0.017     | 0.008      | 0.006      | 0.005       |

It will be noted that the improvement in power factor of cotton having 55% combined acetic acid content over cotton having 29% combined acetic acid content is much less at 1000 cycles than at 50 cycles, so that it would be expected that at radio frequencies little or no improvement with respect to the original well washed cellulose would be obtained.

Under dry conditions the improvement in power factor for lower frequencies of alternating current obtained by partial esterification was found to be so small as to be often lost in the margin of experimental error, and it was only by averaging numbers of samples that the improvement could be established with certainty.

This is illustrated by the following table showing power factors under dry conditions:

|                                                     | 50 cycles | 400 cycles | 800 cycles | 1000 cycles |
|-----------------------------------------------------|-----------|------------|------------|-------------|
| Washed cotton.....                                  | 0.0034    | 0.005      | 0.006      | 0.006       |
| Cotton having 29% combined acetic acid content..... | 0.003     | 0.005      | 0.005      | 0.005       |
| Cotton having 55% combined acetic acid content..... | 0.003     | 0.004      | 0.005      | 0.005       |

These figures heightened the impression that under dry conditions no improvement at all in power factor for radio frequencies would be secured by acetylating to a high degree.

5 The increase in electric resistance to direct current obtained by esterifying the cellulose beyond the diacyl stage is not generally sufficiently great to justify the process being carried to that extent, but for special purposes the higher values 10 of direct current resistance under humid conditions that may be obtained by esterifying beyond the diacyl stage have led to such processes being carried out even up to the stage of full esterification. For these processes it is necessary to add to 15 the bath an inert diluent such as toluene to prevent excessive swelling of the material and tendering of the yarn.

With the development of the transmission of higher and higher frequencies over electric cables it has become necessary to use electric insulating material that has high electric resistance and low power factor at higher frequencies than have hitherto been taken into consideration. It is only recently, however, that measurements of 20 A. C. resistance and power factor at frequencies 25 higher than about 1 kc. could be carried out with accuracy, particularly on yarn materials.

The single figure of the drawing shows a coaxial cable insulated in accordance with my invention.

According to this invention we provide an electric conductor for the transmission of electric currents having a frequency of 10 kc. and above (which may be superimposed on D. C. currents 30 or on A. C. currents of lower frequency) insulated by native cellulosic material that has been esterified up to and beyond the diacyl stage without loss of tensile strength sufficient to prevent the material from being applied to the conductor 35 in the manner in which it is usually applied, including native cellulosic materials that have been fully esterified without such loss of tensile strength.

For the purpose of this invention the only cellulose esters to be considered are those of carboxylic acids having from 2-5 carbon atoms, as these are the esters that we have so far found suitable, but the invention must be taken to include mixed cellulose esters of such acids.

40 The carrying out of measurements of electric 45 resistance and power factor at high frequencies has verified the opinions previously formed as to the behaviour at high frequencies of the lower esterified celluloses. We have found however that cellulose esters of carboxylic acids having from 50 55 2-5 carbon atoms prepared by esterifying native cellulose up to and beyond the diacyl stage without appreciable tendering of the fibres possess very low power factors for the higher frequencies 60 of alternating current and that the increase of

power factor with increase of frequency is small compared with that of the lower esterified materials. The power factor of acylated cotton yarn having 55% combined acetic acid content for example, increases from 0.005 at 1 kc. to 0.008 at 1000 kc. under conditions of ordinary atmospheric humidity whilst the power factor of acylated cotton yarn having 29% combined acetic acid content increases under similar conditions from 0.009 at 1 kc. to 0.015 at 1000 kc. Moreover, contrary to previous experience with lower combined acetic contents, a large improvement in power factor at 1000 kc. even under dry conditions has been obtained by esterification of cotton to a combined acetic acid content of 55% and above. Thus the power factor of acylated cotton yarn having 29% combined acetic acid content is 0.013 for 1000 kc. under dry conditions, but that of cotton yarn acylated to 55% acetic acid content is only 0.005. Also, under dry conditions the power factor of cotton acylated to 55% is nearly constant between 1 kc. and 1000 kc., only rising from .0045 to .0055 over this wide frequency range.

By carrying the acylation still further to a combined acetic acid content of 60 to 62% a still lower power factor and a flatter frequency power factor characteristic can be obtained, i. e. at 1 kc. 0.004 and at 1000 kc. 0.0043.

The present invention is of particular value when applied to coaxial conductor electric cables for the transmission of a very wide frequency band, and more especially to cables constructed as shown in U. S. patents to Wentz Nos. 2,018,477 issued October 22, 1935 and 2,038,973, issued April 28, 1936 and in the figure of the drawing in which, according to the present invention, the insulating separator or separators is or are composed of native cellulose esterified to or beyond the diacyl stage. By the use of such material for the separator we have been able to raise the upper limit of the frequency band satisfactorily transmitted in this type of cable as compared with cables wherein lower esterified cellulose has been used as the separator. For example, in a certain type of coaxial cable insulated with cotton acylated to 29% combined acetic acid content, the attenuation for a frequency of 2½ megacycles was 7.0 decibels per mile. When insulation consisting of cotton acylated to 55% combined acetic acid content was used, the attenuation for this frequency was 5.9 decibels per mile.

In the preparation of highly esterified cellulose several different catalysts have different effects upon the electric insulating properties of the final product but these effects are not of such great importance with respect to the properties in relation to alternating current under dry or moderately humid conditions as they are with respect to the resistance as measured with direct current. For some purposes however, it is desirable to use as the insulating material for electric cables material that has not only a high electric resistance and low power factor when measured with alternating current but also a high electric resistance to direct current under humid conditions. For these purposes additional precautions, such as are described in the specification of British Patent 489,928 by Lovell Strange Eaton Ellis as a communication from Chemical Works formerly Sandoz, must be taken in the esterification process. In particular we have found that when sulphuric acid is used as a catalyst, not only is there a decrease in tensile strength of the esterified ma-

terial, but the direct current resistance under humid conditions is very much lower, compared in each case with similar material for the preparation of which the zinc chloride type of catalyst is used. The alternating current power factors under dry and moderately humid conditions, on the other hand, are equal to that of material using the zinc chloride type of catalyst. Under conditions of high humidity, however, even the alternating current power factor is adversely affected, and accordingly for use in such conditions it is desirable that material prepared with sulphuric acid as a catalyst should be avoided.

#### Example 1

15 The constitution of the bath for the preparation of materials to be used with electric conductors according to the invention can be:—  
Percent  
20 Toluene, petrol or other inert diluent 50  
Acetic anhydride 25  
Acetic acid 20  
Zinc chloride 5

25 The cellulose must be immersed in this bath for a sufficient length of time to allow the desired degree of esterification to take place, this being about 40 hours at a temperature of from 40-50° C. in the case of cotton, which gives a material having a combined acetic acid content of about 55%. After this the acylated yarn is taken out of the acylation mixture, carefully hydro-extracted and washed.

#### Example 2

35 Cotton yarn or other cotton material purified by bucking and bleaching is carefully washed, then dried to a moisture content of about 1-2% and immersed for two hours at 40° C. in acetic acid containing about 2% of water, then taken 40 out, pressed to 60% of adherent liquid and then immersed in the following bath:  
Percent  
Benzene, petrol or other inert diluent 65  
Acetic acid anhydride 15  
45 Glacial acetic acid 15  
Anhydrous zinc chloride 5

50 The acylation is carried out so as to allow the circulation of the acylating liquor through cellulose material for 25 hours, at a temperature of 40° C., which in the case of cotton yarn purified as above gives a combined acetic acid content of 56%. After this time the acylated yarn is carefully washed, the degree of washing being controlled by measuring the electrical conductivity of the wash water and finally hydro-extracted and dried at about 90° C.

I claim:

1. An electric conductor forming part of a cable for transmission of frequencies of 10 kc. or over, and insulation for said conductor having sufficient tensile strength to permit the material to be applied in the usual manner, and having a power factor less than .01 at the frequency range specified, comprising native cellulose material esterified at least to the diacyl stage to form an ester or esters of a carboxylic acid or acids having from two to five carbon atoms.

2. Electric conductor as claimed in claim 1 in which the esterified cellulose material is free from ions derived from sulphuric acid.

ARCHIBALD ALAN NEW.